

# United States Patent Office

3,000,956  
Patented Sept. 19, 1961

1

3,000,956

ALIPHATIC NITRAZA POLYNITRO COMPOUNDS  
Milton B. Frankel, Pasadena, Calif., assignor to Aerojet-General Corporation, Azusa, Calif., a corporation of Ohio  
No Drawing. Filed Oct. 28, 1957, Ser. No. 694,692  
20 Claims. (Cl. 260—583)

This invention relates to new compositions of matter and a method for their preparation. In particular, this invention relates to bis-mineral acid salts of aliphatic nitraza polynitro diamines having the general formula:



and to their corresponding free diamines; wherein X is an anion of a strong mineral acid, the A radicals are alkylene radicals which may be the same or different, and n is a small whole number from 1 to 3, inclusive.

The diamines of the present invention condense with  $\beta$ -geminal polynitro alcohols, such as 2,2,2-trinitroethanol, to form nitramine compounds, as more fully disclosed in assignee's copending U.S. patent application Serial No. 451,705, filed August 23, 1954, now abandoned. The nitramine compounds thus formed react with nitric acid to yield high energy nitramines, as more fully disclosed in assignee's copending U.S. patent application Serial No. 641,437, filed February 19, 1957.

The high energy nitramines prepared from the diamines of this invention by the method described above are useful as high explosives and can be used in any conventional explosive missile, projectile, rocket, or the like, as the main explosive charge. An example of such a missile is disclosed in United States Patent No. 2,470,162, issued May 17, 1949. One way of using the high explosives in a device such as that disclosed in United States Patent No. 2,470,162 is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time-fuse mechanism firing a detonating explosive such as lead azide or mercury fulminate.

The novel inorganic acid salts of the present invention are prepared by reacting an aliphatic nitraza polynitro diisocyanate with a dilute aqueous solution of a strong mineral acid, in accordance with the general reaction scheme set forth below:



wherein X, A, and n are as defined above.

The corresponding free nitraza diamines are generated from the novel mineral acid salts of this invention by neutralizing the salts with inorganic basic salts of alkali or alkaline earth metals, such as hydroxides or carbonates, or weak organic acid salts, such as acetates, of alkali or alkaline earth metals. For reasons of convenience and economy, I prefer to use sodium hydroxide as the amine generating agent, but other suitable generating agents, such as calcium hydroxide, magnesium

2

hydroxide, sodium carbonate, lithium acetate, strontium formate, etc., can be employed for this purpose.

To more clearly illustrate this invention, the following example is presented. It is to be understood, however, that this example is presented merely as a means of illustration, and is not intended to limit the scope of the invention in any way.

## EXAMPLE

### 10 Preparation of the bis-nitric acid salt of 3,3,5,7,7-penta-nitro-5-aza-1,9-nonane diamine

In a round-bottom flask fitted with a reflux condenser, 3,3,5,7,7-penta-nitro-5-aza-1,9-nonane diisocyanate was heated with a ten-fold excess of 35% nitric acid on a steam bath for a period of 3 hours. The solution was evaporated to dryness in *vacuo* leaving a quantitative yield of the bis-nitric acid salt of 3,3,5,7,7-penta-nitro-5-aza-1,9-nonane diamine. Upon recrystallization from concentrated nitric acid the product exhibited a M.P. of 175-180° C. The elemental analysis of the product is as follows:

Calculated for  $\text{C}_8\text{H}_{18}\text{N}_{10}\text{O}_{16}$ : percent C, 18.83; percent H, 3.56; percent N, 27.45. Found: percent C, 18.95; percent H, 3.88; percent N, 27.10.

The explosive power of this compound was calculated as follows:

|                        |     |              |
|------------------------|-----|--------------|
| 30 Lead block value    | 135 | T.N.T. = 100 |
| Ballistic mortar value | 144 | T.N.T. = 100 |

As already indicated, a dilute mineral acid is employed for the reaction of the present invention. By dilute acid, as the term is used herein, is meant an aqueous solution of acid, preferably from about 30 to about 85% concentration. The reaction of this invention is a vigorous one, and I have found that optimum control can be exercised when an acid of about 35% concentration is employed in excess, particularly where the mineral acid used is nitric acid. The excess acid acts as a diluent or solvent, and thereby effects moderation of the reaction.

The reaction temperature is not critical in the practice of this invention, the only effect of temperature variation being a corresponding increase or decrease in reaction rate. I have found, however, that elevated reaction temperatures, such as those from ambient to about 100° C., result in particularly favorable reaction rates, and that the reaction proceeds most efficaciously at steam bath temperature.

The diisocyanates used as starting materials in this invention are obtained by reacting diacyl halides, such as 6-aza-4,4,6,8,8-pentanitro-1,11-undecanedioyl chloride, with alkali or alkaline earth metal azides, such as sodium azide, to form the corresponding nitraza azides, and then heating said nitraza azides to effect rearrangement to the desired diisocyanate form. Treating the above-mentioned diacyl halide as described results in the formation of 3,3,5,7,7-penta-nitro-5-aza-1,9-nonane diisocyanate starting materials is more fully described in assignee's copending U.S. patent application Serial No. 451,707, filed August 23, 1954, now abandoned. The nitraza diacyl halides are prepared from their corresponding esters, obtained by the condensation of geminal polynitrohydroxy esters in the presence of ammonia or an amine followed by nitration of the condensation products, as disclosed in assignee's copending application No. 416,382, filed March 15, 1954, now abandoned.

The diisocyanates wherein n is greater than 1 are prepared in accordance with the above procedure by condensing a hydroxy polynitro ester with the amine, obtained from an isocyanate previously prepared as described, and

subsequently forming the acid halide and reacting it with sodium azide to form the desired isocyanate.

The strong mineral acid with which the diisocyanate is reacted in the practice of this invention is preferably nitric acid or perchloric acid, since when either of these acids is employed, the resulting salt is useful as a high explosive in addition to having utility as an intermediate in the preparation of other high explosive compounds, as described above. However, other strong mineral acids, such as hydrochloric acid, sulfuric acid, or the like, can be employed for purposes of this invention if desired.

It will be appreciated that a wide variety of bis-inorganic acid salts of aliphatic nitraza polynitro diamines can be prepared in accordance with the method of my invention. For example, 2,2,5,8,8-pantanitro-5-aza-1,9-nonane diisocyanate; 2,2,5,9,9-pantanitro-5-aza-1,13-tridecane diisocyanate; 3,3,6,9,9,12,15,15-octanitro-6,12-diaza-1,17-heptadecane diisocyanate; and 3,3,5,7,7,10,12,12-octanitro-5,10-diaza-1,14-tetradecane diisocyanate react with strong mineral acids, such as nitric acid or perchloric acid, in dilute aqueous solutions, to produce the corresponding mineral acid salts, such as the nitric acid or perchloric acid salts, of 2,2,5,8,8-pantanitro-5-aza-1,9-nonane diamine; 2,2,5,9,9-pantanitro-5-aza-1,13-tridecane diamine; 3,3,6,9,9,12,15,15-octanitro-6,12-diaza-1,17-heptadecane diamine; and 3,3,5,7,7,10,12,12-octanitro-5,10-diaza-1,14-tetradecane diamine, respectively. The free nitraza diamines can be readily generated from these acid salts through neutralization thereof with an inorganic basic salt or a weak organic acid salt of an alkali or alkaline earth metal, as taught herein.

It is apparent that the strong mineral acid salts of any member of this series of aliphatic nitraza polynitro diamines can be obtained by merely reacting the appropriate diisocyanate with dilute mineral acid, in accordance with the example set forth above. It is equally apparent that the free diamines can be generated from the mineral acid salts thereof through neutralization with an inorganic basic salt or a weak organic acid salt of an alkali or alkaline earth metal, as taught herein.

This application is a continuation-in-part of my pending U.S. patent application Serial No. 451,708, filed August 23, 1954, now abandoned.

I claim:

1. As compositions of matter, nitraza compounds selected from the group consisting of aliphatic nitraza polynitro diamines having the formula:



wherein the A radicals are lower alkylene and n is a small whole number from 1 to 3, inclusive; and strong mineral acid salts thereof.

2. As compositions of matter, the aliphatic nitraza polynitro diamines having the formula:



wherein the A radicals are lower alkylene and n is a small whole number from 1 to 3, inclusive.

3. As compositions of matter, the strong mineral acid salts of aliphatic nitraza polynitro diamines having the formula:



wherein X is an anion of a strong mineral acid, the A radicals are lower alkylene and n is a small whole number from 1 to 3, inclusive.

4. As compositions of matter, the bis-nitric acid salts

of aliphatic nitraza polynitro diamines having the formula:



wherein the A radicals are lower alkylene and n is a small whole number from 1 to 3, inclusive.

5. As compositions of matter, the bis-perchloric acid salts of aliphatic nitraza polynitro diamines having the formula:



wherein the A radicals are lower alkylene and n is a small whole number from 1 to 3, inclusive.

6. As a composition of matter, the bis-nitric acid salt of 3,3,5,7,7-pantanitro-5-aza-1,9-nonane diamine having the structural formula:



7. As a composition of matter, the bis-nitric acid salt of 2,2,5,8,8-pantanitro-5-aza-1,9-nonane diamine having the structural formula:



8. As a composition of matter, the bis-nitric acid salt of 2,2,5,9,9-pantanitro-5-aza-1,13-tridecane diamine having the structural formula:



9. As a composition of matter, the bis-nitric acid salt of 3,3,6,9,9,12,15,15-octanitro-6,12-diaza-1,17-heptadecane diamine having the structural formula:



10. As a composition of matter, the bis-nitric acid salt of 3,3,5,7,7,10,12,12-octanitro-5,10-diaza-1,14-tetradecane diamine having the structural formula:



11. The method of preparing a strong mineral acid salt of nitraza compounds selected from the group consisting of aliphatic nitraza polynitro diamines having the formula:



which comprises reacting an aliphatic nitraza polynitro diisocyanate having the formula:



with dilute mineral acid; wherein the A radicals are lower alkylene and  $n$  is a small whole number from 1 to 3, inclusive.

12. The method of preparing bis-nitric acid salts of aliphatic nitraza polynitro diamines having the formula: 5



which comprises reacting dilute nitric acid with an aliphatic nitraza polynitro diisocyanate having the formula: 10



wherein the R radicals are lower alkylene and  $n$  is a small whole number from 1 to 3, inclusive.

13. The method of preparing bis-perchloric acid salts of aliphatic nitraza polynitro diamines having the formula: 15



which comprises reacting dilute perchloric acid with an aliphatic nitraza polynitro diisocyanate having the formula: 20



wherein the A radicals are lower alkylene and  $n$  is a small whole number from 1 to 3, inclusive.

14. The method of preparing the bis-nitric acid salt of 3,3,5,7,7-pentanitro-5-aza-1,9-nonane diamine, which comprises reacting 3,3,5,7,7-pentanitro-5-aza-1,9-nonane diisocyanate with dilute nitric acid.

15. The method of claim 11 in which the dilute mineral acid has a concentration of from about 30% to about 85%.

16. The method of claim 12 in which the dilute nitric acid has a concentration of about 35%.

17. The method of preparing bis-nitric acid salts of aliphatic nitraza polynitro diamines having the formula:



which comprises reacting an aliphatic nitraza polynitro diisocyanate having the formula:



with 35% nitric acid, in the presence of excess dilute nitric acid and at an elevated temperature; wherein the A radicals are lower alkylene and  $n$  is a small whole number from 1 to 3, inclusive.

18. The method of preparing aliphatic nitraza polynitro diamines having the formula:



which comprises reacting dilute mineral acid with an aliphatic nitraza polynitro diisocyanate having the formula:



30 wherein the R radicals are lower alkylene and  $n$  is a small whole number from 1 to 3, inclusive, to form a bis-mineral acid salt of a diamine and neutralizing the salt with another salt selected from the group consisting of inorganic basic salts of alkali and alkaline earth metals and weak organic acid salts of alkali and alkaline earth metals.

35 19. The method of preparing the bis-perchloric acid salt of 2,2,5,8,8-pentanitro-5-aza-1,9-nonane diamine, which comprises reacting 2,2,5,8,8-pentanitro-5-aza-1,9-nonane diisocyanate with dilute perchloric acid.

40 20. The method of claim 17 in which the reaction is conducted at about 100° C.

No references cited.